

## UNITED STATES PATENT OFFICE

2,463,483

PROTECTION OF METALLIC OBJECTS BY  
GALVANIC ACTIONJean Frasch, also known as Herbert Manfred  
Freud, Clichy, FranceNo Drawing. Application January 17, 1940, Se-  
rial No. 314,349. In France January 31, 1939

9 Claims. (Cl. 204—56)

1

In the copending U. S. patents application Serial Number 297,191 entitled "Improvements in process for the protection of magnesium and its alloys," filed on September 29, 1939, which has became abandoned, the present inventor has described a process for producing a coating resistant to corrosion on magnesium-base objects, which consisted in employing an acid bath characterised by the presence of an ion containing the element manganese. In the aforesaid patent application it is stated that the invention is preferably carried out by means of alternating current, but that it is also possible to procure the protective coating in question by purely chemical means. In this latter case the chemical action is defined as being obtained by immersion in the bath of the magnesium-base object to be protected without the said object forming any part of an electric circuit through which current passes.

The inventor on continuing his researches has now discovered that the presence in the bath of an ion containing the element manganese is capable of giving rise to galvanic phenomena resulting in the deposition not only on magnesium and its alloys but also on other metals, of a protective coating more resistant to corrosion than any which have heretofore been obtained. In other words if one connects, in the absence of any extraneous source of electric current, the object to be treated to a second electrode in the bath by means of an electric conductor outside the bath, an electric current is set up which ceases if the electric connection is broken. The system functions as a primary cell, and one obtains in this way, the aforementioned excellent coating so highly resistant to corrosion.

The new invention consequently consists in immersing the metallic object to be protected, after suitable degreasing and pickling, in a bath containing ions wholly or partially constituted of manganese. The said metallic object, which may for example be composed of a magnesium-base metal, is then electrically connected, as explained above, to a second electrode composed of a more noble metal or element, such for instance as lead, iron or especially carbon, without the adjunction of any extraneous source of current. A galvanic current is at once set up, accompanied by a deposit of an oxide of manganese on the magnesium-base electrode. As has been stated, this coating is particularly resistant to corrosion.

The manganese may be present in the bath either in the form of manganese ions formed by the dissociation of a manganous salt, or in the form of manganate or permanganate ions. It is

2

particularly advantageous that the ion containing the element manganese should be associated with chromate or bichromate ions, as for instance in  $MnCr_2O_7$ .

5 The inventor has further discovered that all soluble manganates and permanganates are capable of giving rise to the above described protective coating, whereas not all soluble manganese salts can be so employed. Thus for instance nitrates, chlorides and sulphates are incapable of forming adequate protective coatings on magnesium-base metals, since they attack the metal. By such attack on the metal, some of the magnesium (from the surface of the magnesium or magnesium base alloy) would become dissolved in the bath, and some of it would be found in the coating produced galvanically in the process, which latter would give a coating of inferior quality.

20 In the case of voluminous metal objects which it is difficult to treat in a bath, the inventor has found that one can replace the immersion in a bath as described above by the apposition on the object to be treated of rags or other absorbent substances impregnated with the desired solution, the said objects to be protected being as before electrically connected to the other electrodes which are also in contact with the said impregnated rags or other absorbent substances.

25 The coating obtained is usually brown, the colour being of varying shades and intensities, and in general, especially in the case of magnesium, does not contain any compound into which the metal or metals to be protected enter. 30 The coating is formed of an oxide or oxides of manganese, which may also be associated with an oxide of metals whose ions are present together with manganese in the bath.

35 The protection afforded by the coating so produced can be still further increased by treatment in a bath of hot paraffin at temperatures of about 150 to 200°C., also by treatment with other hot heavy hydrocarbons. The inventor has discovered to his surprise that if a metallic object, for example an object composed of a magnesium alloy, is treated as set forth above and then dipped in a bath of hot paraffin, a violent chemical reaction takes place, as is evidenced by a copious evolution of gas. At the same time the structure 45 of the protective coating is changed, and the colour deepens to black. It appears that the oxide or oxides forming the protective film will be chemically acted upon by the paraffin, at the temperatures stated, and hydrated compounds 50 will undergo dehydration.

The following examples, which are given by way of example only, and which must not therefore be construed in any limiting spirit, will make clear exactly and in what way the above invention is to be carried out.

*Example 1.*—A piece of sheet composed of a magnesium alloy containing 1.5% manganese, is cleaned mechanically and immersed for one hour in a 1% solution of  $KMnO_4$ , and at the same time connected electrically to a second electrode of carbon. The temperature of the solution is maintained at  $60^\circ C$ . One obtains a light brown film of an oxide of manganese.

*Example 2.*—An object composed of a magnesium-alloy containing 3% Al and 1% Zn which object has been forged, is pickled in a solution of chromic acid and immersed at room temperature for 4 hours in a 10% solution of  $MnCr_2O_7$ , and at the same time connected electrically to a second electrode of carbon. One obtains a dark brown coating, which takes on a black aspect after treatment in a bath of hot paraffin at  $180^\circ C$ . The film contains an oxide of manganese together with an oxide of chromium.

*Example 3.*—A cast object composed of magnesium alloy containing 10% Al, is first pickled in nitric acid and then immersed for 2 hours at room temperature in a solution made by dissolving 50 grams of  $CrO_3$ , 10 grammes of  $KMnO_4$  and 50 grammes of  $MnCO_3$  in 1 litre of water, the said object being at the same time electrically connected to a second electrode of iron. The film obtained is grey.

*Example 4.*—An object composed of semi-mild steel, after previous picking in  $H_2SO_4$ , is immersed for half an hour at  $40^\circ C$ . in a solution obtained by dissolving 100 grammes of  $MnCO_3$  in a litre of water containing 70 grammes of  $CrO_3$ , the said object being at the same time connected electrically with a second electrode of lead. One obtains a grey film which turns black after treatment in hot paraffin.

The coatings so formed are very adherent, and can be obtained very thick if one continues the galvanic treatment for a sufficient length of time. The coating is moreover of substantially uniform thickness and character irrespective of the shape of the object treated. This is true even for the interior of angles or tubes in contradistinction to the well known difficulty of obtaining uniform deposits on such parts in the case of the anodic processes of protection habitually employed. It is highly probable that this result is due to the nature of the current giving rise to the deposit, this current being galvanic and not electrolytic in origin; in other words the process itself produces the electric current necessary to form the deposit, instead of consuming an electric current extraneously produced.

The above invention also covers as new industrial products all metallic objects, and in particular objects made of magnesium-base metals, on which coatings composed principally of an oxide of manganese have been deposited, either as such or when subsequently treated in a bath of hot paraffin or other hydrocarbon, the galvanic baths serving to put the said invention into effect and the protective coating itself so obtained.

I claim:

1. A process for protecting metallic objects composed of a substance selected from the group consisting of magnesium and alloys containing

magnesium as their major constituents, by making the object to be protected the anode, in a galvanic battery having a cathode more noble than magnesium and having an electrolyte consisting essentially of an aqueous solution of at least one compound selected from the group consisting of manganates, permanganates and manganese bichromate, electrically connecting said anode and said cathode outside said bath, and allowing a galvanic current to flow, in said solution, from said anode to said cathode until a protective film of substantial thickness is formed on said anode, removing said anode from said solution and washing same, all without supplying any electric current from the outside of said galvanic cell.

2. Process according to claim 1 in which the electrolyte is an aqueous solution of a manganate.

3. Process according to claim 1 in which the electrolyte is an aqueous solution of a permanganate.

4. Process according to claim 1 in which the electrolyte consists essentially of an aqueous solution of manganese bichromate.

5. An article formed of a substance selected from the group consisting of magnesium and magnesium alloys containing magnesium as the major component, and having a coating consisting essentially of an oxide of manganese and an oxide of chromium, which coating is brown to black in color and which coating is devoid of magnesium compounds, such coating being very adherent to the magnesium and very resilient to corrosion, and of substantially uniform thickness.

6. A process as in claim 1, in which the electrolyte is a solution of  $MnCr_2O_7$  of about 10% concentration.

7. A process as in claim 1, in which the electrolyte is a solution of permanganate of about 1% concentration.

8. A process as in claim 1, in which the electrolyte is a solution of manganese bichromate and a permanganate.

9. A process as in claim 1, in which the electrolyte is an aqueous solution made by adding 50 gr.  $MnCO_3$ , 50 gr.  $CrO_3$  and 10 gr.  $KMnO_4$  to each liter of water.

JEAN FRASCH.

50 Also Known as *Herbert Manfred Freud*.

#### REFERENCES CITED

The following references are of record in the file of this patent:

#### UNITED STATES PATENTS

| Number    | Name          | Date           |
|-----------|---------------|----------------|
| 737,882   | Strecker      | Sept. 7, 1903  |
| 1,552,591 | Batenburg     | Sept. 8, 1925  |
| 1,952,850 | Kochler       | Mar. 27, 1934  |
| 1,974,435 | Schulz et al. | Sept. 25, 1934 |
| 2,052,962 | Booe          | Sept. 1, 1936  |
| 2,138,023 | Buzzard       | Nov. 29, 1938  |
| 2,203,670 | Buzzard       | June 11, 1940  |
| 2,206,028 | Buzzard       | July 2, 1940   |
| 2,224,528 | Sutton et al. | Dec. 10, 1940  |

#### FOREIGN PATENTS

| Number  | Country       | Date          |
|---------|---------------|---------------|
| 493,935 | Great Britain | Oct. 17, 1938 |
| 702,266 | France        | Jan. 20, 1931 |
| 471,053 | Germany       | Feb. 6, 1929  |

**Certificate of Correction**

March 1, 1949.

Patent No. 2,463,483.

JEAN FRASCH, also known as HERBERT MANFRED FREUD

It is hereby certified that errors appear in the printed specification of the above numbered patent requiring correction as follows:

Column 4, line 1, claim 1, for the word "constituents" read *constituent*; line 33, claim 5, for "resilient" read *resistant*; and that the said Letters Patent should be read with these corrections therein that the same may conform to the record of the case in the Patent Office.

Signed and sealed this 17th day of May, A. D. 1949.

[~~SEAL~~]

THOMAS F. MURPHY,  
*Assistant Commissioner of Patents.*